

[54] **FERRITIC ALLOY WITH HIGH TEMPERATURE STRENGTH CONTAINING DISPERSED INTERMETALLIC TiSi**

[75] Inventors: **Philip M. Giles**, Bethlehem; **Halle Abrams**, Allentown; **Arnold R. Marder**, Bethlehem, all of Pa.

[73] Assignee: **Bethlehem Steel Corporation**, Bethlehem, Pa.

[22] Filed: **July 20, 1973**

[21] Appl. No.: **381,288**

[52] U.S. Cl. .... **75/124**, 75/128 C, 75/128 T

[51] Int. Cl. .... **C22c 39/04**

[58] Field of Search .... **75/124, 128 C, 128 T**

[56] **References Cited**

UNITED STATES PATENTS

3,660,173 5/1972 Matsuho ..... 75/124  
3,676,109 7/1972 Cooper ..... 75/124

Primary Examiner—L. Dewayne Rutledge  
Assistant Examiner—Arthur J. Steiner  
Attorney, Agent, or Firm—Joseph J. O'Keefe; William B. Noll

[57] **ABSTRACT**

An iron-aluminum ferritic alloy characterized by high-temperature strength, resulting from the precipitation of a fine TiSi intermetallic type precipitate of high thermal stability, and high-temperature oxidation-resistance under conditions of cyclic heating at temperatures up to about 2,500° F. said alloy consists essentially of, by weight, up to about 0.1% carbon, from about 4.0 to about 8.2% aluminum, about 0.2 to 4.0% silicon, about 0.05 to 2.0% titanium, with a preferred silicon/titanium ratio between about 1.0 to 4.0, and the balance iron, incidental impurities and additions which do not materially affect the attainment of the desired properties.

**10 Claims, 1 Drawing Figure**



**FERRITIC ALLOY WITH HIGH TEMPERATURE  
STRENGTH CONTAINING DISPERSED  
INTERMETALLIC TiSi**

**CROSS-REFERENCES TO RELATED  
APPLICATION**

This invention is an improvement over the high-temperature oxidation-resistant ferrous alloy disclosed and claimed in copending application, Ser. No. 275,650, assigned to the assignee herein.

**BACKGROUND OF THE INVENTION**

This invention relates to a high-strength, low-cost iron-aluminum ferritic alloy, characterized by a microstructure containing a fine TiSi intermetallic type precipitate dispersed uniformly throughout the matrix of the grains thereof. The alloy also possesses high-temperature oxidation-resistance, a characteristic ideally suited for application where thermal shock, such as cyclic heating and cooling, are experienced. While not intending to unduly limit this invention, applications which can take advantage of the properties hereof are high temperature exhaust systems in automobiles, jet engines, and in the petrochemical industry.

Heretofore, high-temperature oxidation-resistant materials were selected from high cost nickel and cobalt superalloys, austenitic stainless steels, or ceramic materials. In an effort to lower cost, the prior art moved to lower or less rich alloys. For example U.S. Pat. No. 1,641,752 teaches a ferrous alloy resistant to oxidation at high temperatures, by including therein a high percentage of aluminum. Specifically, said alloy contains from 12 to 20% aluminum, and about 1 to 5% of a grain refining material, among which are included titanium and chromium. The high-temperature oxidation-resistance is due at least in part to the formation of a protective coating of oxide of the aluminum on the exposed surfaces of the ferrous alloy. However, such alloys are of limited suitability under cyclic heating and cooling conditions wherein thermal shock results in flaking and spalling of the oxide coating. Accordingly, one of the critical requirements of a suitable alloy is its ability to resist such flaking and spalling.

A more recent development covering high-temperature oxidation-resistant alloys is described in U.S. Pat. No. 3,192,073. This patent teaches a method for making an iron-aluminum alloy product fortified for high-temperature environments by the application to the said product of an aluminum coating, followed by a high temperature anneal to diffuse said coating into the alloy product. The oxidation-resistance of the coated and heat treated product is enhanced by the further development of iron-aluminum compounds near the surface thereof. In other words, a protective layer or enriched case is formed about the said product. Over and above the costly treatments for coating and diffusion annealing, there is a serious question of whether such a product could withstand the cyclic heating and cooling which is incidental to many industrial applications. For example, the material of the latter patent is characterized by an aluminum gradient between the coating and core, and as a result would have different densities and coefficients of expansion. Thermal cracks could develop from said cyclic treatments, as well as an eventual deterioration thereof due to continued diffusion and depletion of the aluminum from the coating.

As is evident from the preceding discussion, iron-aluminum alloys have served as a base alloy for developing high-temperature oxidation-resistant alloys. U.S. Pat. No. 3,698,964, represents a further effort in this direction. Briefly, the alloy of said patent is an iron base alloy containing chromium and aluminum and/or silicon. More specifically, the alloying additions thereto are on the order of from 1 to 5%. The improved oxidation-resistance, or decrease in weight gain with temperature, is attributed to the formation of alumina, or a complex oxide of iron and aluminum. While such an alloy appears to exhibit superior oxidation-resistance when compared to a Type 301 austenitic stainless steel, no mention is made as to its high temperature strength.

15 In contrast to this, the present invention teaches a ferritic alloy which is not only oxidation-resistant at elevated temperatures, but possesses high strength in conjunction therewith.

**SUMMARY OF THE INVENTION**

The present invention relates to a high-strength iron-aluminum ferritic alloy which is not only resistant to oxidation at high temperatures, but is resistant to surface flaking and spalling when subjected to thermal shocking as a result of cyclic heating and cooling. More particularly, said invention covers an alloy consisting essentially of, by weight, up to about 0.1% carbon, about 4.0 to 8.2% aluminum, up to about 10.5% chromium, about 0.2 to 4.0% silicon, about 0.05 to 2.0% titanium, with a preferred silicon titanium ratio between about 1.0 to 4.0 and the balance iron, incidental impurities and additions which do not materially affect the attainment of the desired properties. The unexpected high-temperature strength is derived from the precipitation at very high temperatures, of a fine TiSi intermetallic type precipitate of high thermal stability, said precipitate being uniformly dispersed throughout the matrix of the grains thereof.

**BRIEF DESCRIPTION OF DRAWING**

The FIGURE is a graph showing the increase or change in strength, over a range of elevated temperatures, for two alloys of this invention (base alloys plus titanium and silicon according to the teachings herein) and base alloys plus no more than one of the elements from the group consisting of silicon, titanium, or an increase in the carbon content.

**DETAILED DESCRIPTION OF PREFERRED  
EMBODIMENT**

This invention is directed to the family of iron-aluminum alloys, more particularly to the wrought ferritic alloys thereof which may be employed in applications where the ability to withstand thermal shock is critical. The alloys hereof are characterized by a combination of high-strength and oxidation-resistance under conditions of cyclic heating at temperatures up to about 1,800° F. Typical applications where the latter conditions prevail are high temperature exhaust systems, such as a thermal reactor in automobiles, jet engines, and in the petrochemical industry. While the mention of same is not intended as a limitation on this invention, it is believed that a brief discussion thereof will help in understanding the significance of this invention and the contributions offered thereby.

Generally, a thermal reactor is a container into which the hot exhaust gases flow from the automotive, jet or

power producing engines, for further combustion. Air is also pumped into the reactor and admixed with said gases. The reactor is generally of sufficient size (chamber volume) to give a long enough residence time of the admixed gases to permit complete combustion of the residual hydrocarbons and carbon monoxide. Since the combustion reaction is so strongly exothermic, temperatures may go as high as 2,200° F., typically about 1,800° F., in a highly oxidizing environment. Thus, the severe conditions of high temperature, oxidizing environment, and intermittent operation (cyclic heating and cooling), call for a material capable of meeting these conditions. The alloys of the present invention not only fulfill these conditions, but accomplish it at a low material cost. That is, as a result of the unexpected increase in strength, less material is required.

The composition of the alloys of this invention fall broadly within the alloying ranges below:

Carbon — up to about 0.1 wt. %

Aluminum — 4.0 to 8.2 wt. %

Chromium — up to about 10.5 wt. %

Silicon — 0.2 to 4.0 wt. %

Titanium — 0.05 to 2.0 wt. %

Iron — balance,

with a preferred silicon/titanium ratio between about 1.0 to 4.0. Within said broad ranges, a preferred composition is one containing at least about 8.0% chromium, aluminum between about 6.0 to 7.0%, titanium between about 0.2 to 1.2%, silicon between about 0.6 to 1.8%, and a titanium/carbon ratio of at least 4.0.

It will be recalled from the data presented in said copending application that there is a general relationship between the performance of the alloys of the type herein under high-temperature conditions to the richness or total alloying content of the alloy. While this general proposition may suggest improved performance with the richer alloys, there are some practical limits due to alloying costs and processing restrictions.

In this regard, the production of wrought strip and sheet by conventional rolling practices requires that the material be sufficiently ductile for said rolling to be effected. In the case of aluminum containing iron base alloys, the ductility thereof drops below a practical level when the aluminum begins to exceed about 8% by weight. Chromium, when added to an Al-Fe alloy, should not exceed about 10% by weight, as the risk of breakage and other processing problems increases. Finally, with respect to carbon it should be kept to a low

believed that the prior art establishes the general performance of the iron-aluminum alloys to resist high-temperature oxidation, while said copending application establishes the specific capabilities of the alloys hereof to perform at temperatures up to about 2,500° F. Accordingly, the data therefrom is incorporated by reference and will not be presented here.

From this then, the significant feature of the present invention becomes the unexpected increase in strength 10 of the alloys as a result of the precipitation of a fine TiSi intermetallic type precipitate of high thermal stability. The synergism resulting from the controlled addition of both titanium and silicon is believed clearly demonstrated from the FIGURE, and TABLE II below. For 15 this demonstration, two base alloys, Alloys A and C of Table I, were tested as to their strength at varying elevated temperatures. To several other alloys having chemistries comparable to the base alloys were added the elements titanium, carbon and/or silicon. The alloy 20 designations with their melt chemistries, by weight percent, are listed below in TABLE I.

TABLE I

| Alloy | Carbon | Chromium | Aluminum | Titanium | Silicon |
|-------|--------|----------|----------|----------|---------|
| 30    | A      | .019     | 9.0      | 6.4      | .51     |
|       | B      | .014     | 10.0     | 6.3      | .84     |
|       | C      | .012     |          | 7.9      | .004    |
|       | D      | .019     | .03      | 7.9      | .007    |
|       | E      | .068     |          | 8.0      | .51     |
|       | F      | .10      |          | 8.1      | .004    |
|       | G      | .023     |          | 8.2      | .35     |

To secure the date of TABLE II, the various alloys listed above were vacuum-induction melted and vacuum-cast into ingot molds resulting in ingots weighing about 400 lbs. After slow cooling to ambient temperatures, the ingots were slowly heated (at least 5 hours) to a soaking temperature between about 2,025° to 35 2,130° F. For the initial hot rolling, the ingots were reduced at about  $\frac{1}{2}$  inches per pass to a plate thickness of about 1 inch. The finishing temperatures varied between about 1,650° to 1,850° F., and from here the 40 plates were slowly cooled to ambient temperatures by burying in sand. Tensile test specimens were then machined from the plates and tensile tests were then performed on the material. Results of the tensile tests are 45 reported in Table II.

TABLE II

| Alloy | TENSILE STRENGTH (KSI) |             |             |             |             |
|-------|------------------------|-------------|-------------|-------------|-------------|
|       | at 1150° F.            | at 1200° F. | at 1400° F. | at 1600° F. | at 1800° F. |
| A     | —                      | 29.5        | 12.0        | 4.5         | 2.5         |
| B     | —                      | 41.5        | 21.5        | 10.0        | 4.5         |
| C     | 29.0                   | —           | 14.0        | 7.0         | 4.4         |
| D     | 37.9                   | —           | 13.8        | 8.2         | 4.3         |
| E     | 37.4                   | —           | 17.6        | 7.3         | 4.7         |
| F     | 36.9                   | —           | 17.0        | 8.0         | 3.2         |
| G     | 42.6                   | —           | 20.7        | 9.2         | 4.9         |

value, preferably less than about 0.04%, typically less than 0.03%. But in no case should it exceed 25% of the titanium.

From the outset of this description, emphasis has been placed on the two principal characteristics of the alloys of this invention; namely, high-temperature oxidation-resistance, and high-temperature strength. It is

65 While TABLE II presents the results in a form as actually measured, a different approach was taken with the FIGURE. For the graphic demonstration, the strength difference between an appropriate base or reference alloy (the particular base alloy is designated on each curve) and the base alloy plus additives was plotted along the ordinate. The base alloy used for Alloy E

was Alloy F as the carbon difference was less than if Alloy C had been used.

The clear beneficial relationship of the combination of titanium and silicon can best be seen from a comparison of Alloys D and E with Alloy G. From TABLE I it will be observed that to the base chemistry of Alloys D and E, only one of the elements titanium and silicon were included. If, for example, the strength increase attributed to each such element individually were added to each other, the result would still fall far short of that actually realized with Alloy G.

This unexpected improvement may best be illustrated by the FIGURE. The curve  $(\sigma_E - \sigma_F)$  represents the difference in strength observed at various temperatures, when the titanium containing Alloy E is contrasted to Alloy F, comparable in all regards except the titanium content. In similar fashion, curve  $(\sigma_D - \sigma_C)$  represents the difference in strength at the varying temperatures between Alloy D and Alloy C. The alloys were comparable except for the 0.61% by weight silicon in the former. By these comparisons it was possible to essentially isolate the effect of the individual element, titanium or silicon, on the high temperature strength of the alloys. By adding together the strength changes at a given temperature, and comparing it to the curve  $(\sigma_G - \sigma_C)$ , it will be seen that the result is not merely additive, but significantly higher than expected. This synergism is attributed to the development of a TiSi intermetallic type precipitate which has been observed in the matrix of the grains thereof.

Transmission electron microscopic examination of the silicon-titanium bearing alloys of this invention revealed a structure containing a very small (100 to 600A), well dispersed, spherical precipitate of very high thermal stability throughout the matrix of the said grains. Although a positive identification of the precipitate could not be made from currently available ASTM file data, the correspondence between the observed pattern and that of the face-centered-cubic  $Fe_3Si$  ( $a_0 = 5.64A.$ ) is quite good. If it is postulated that some of the iron atoms are replaced by the larger titanium atoms (the radii of the atoms are 1.26 A. for iron versus 1.49 A. for titanium) it becomes very reasonable to believe that the observed precipitate is of the form  $(Fe, Ti)_3Si$  with an  $a_0 = 5.80A.$  and with a face-centered-cubic

45

structure.

Thus, by the discovery of the unique strengthening mechanism attributed to the development of said TiSi intermetallic type precipitate, a high temperature strength version of the iron-aluminum ferritic alloys evolved.

We claim:

1. A high temperature high strength ferritic alloy characterized by a microstructure containing a small, well dispersed, spherical TiSi type intermetallic precipitate and consisting essentially of, by weight, up to about 0.1% carbon, from about 4.0 to about 8.2% aluminum, up to about 10.5% chromium, from about 0.2 to about 4.0% silicon, from about 0.05 to about 2.0% titanium, where the silicon content is at least equal to the titanium content to insure the development of said precipitate, with the balance iron.
2. The ferritic alloy claimed in claim 1 wherein the silicon/titanium ratio is between 1.0 to about 4.0.
3. The ferritic alloy claimed in claim 1 wherein the carbon content is less than about 0.04%.
4. The ferritic alloy claimed in claim 3 wherein the maximum carbon content is 0.03%.
5. A ferritic alloy characterized by high temperature strength and consisting essentially of, by weight, up to about 0.1% carbon, from about 6.0 to about 7.0% aluminum, from about 8.0 to about 10.5% chromium, from about 0.6 to about 1.8% silicon, from about 0.2 to about 1.2% titanium, where the silicon content is at least equal to the titanium content, with the balance iron.
6. The ferritic alloy claimed in claim 5 wherein the silicon/titanium ratio is between 1.0 to about 4.0.
7. The ferritic alloy claimed in claim 5 wherein the carbon content is less than about 0.04%.
8. The ferritic alloy claimed in claim 7 wherein the maximum carbon content is 0.03%.
9. The ferritic alloy claimed in claim 5 wherein the microstructure is characterized by a structure containing a small, well dispersed, spherical intermetallic precipitate.
10. The ferritic alloy claimed in claim 5 wherein said precipitate is a TiSi type intermetallic precipitate.

\* \* \* \* \*